

3,729,308

## IRON NICKEL CHROMIUM ALLOYS

Herbert L. Eiselstein and James C. Hosier, Huntington,  
W. Va., assignors to The International Nickel Company, Inc., New York, N.Y.  
No Drawing. Filed July 21, 1970, Ser. No. 56,977  
Int. Cl. C22c 39/20

U.S. Cl. 75—128 E

10 Claims

## ABSTRACT OF THE DISCLOSURE

Iron-base alloys for sheathing electric heater elements include specially proportioned amounts of nickel (about 15% to about 23%), chromium (about 17% to about 23%), silicon (about 0.3% to about 1.5%) and cerium (an effective amount up to about 0.05%) to assure high oxidation resistance and good corrosion resistance.

This invention is directed to improved oxidation and corrosion resistant low cost iron-base alloys particularly suitable for use as electric heater element sheathing.

One type of electric heater element comprises a resistance conductor which is enclosed in a tubular metal sheath, with the resistance conductor embedded in and supported in spaced relation to the sheath by a densely compacted layer of refractory, heat-conducting, electrically insulating material. The resistance conductor may be a helically wound wire member and the refractory insulating material may be granular magnesium oxide (MgO).

A commercial alloy which is currently used as sheathing material is an iron-base alloy which nominally contains, by weight, 32.5% nickel, 21% chromium, and small amounts of carbon, manganese, sulfur, silicon, copper, aluminum and titanium. While this commercial alloy has performed satisfactorily in the heater sheathing application, an alloy exhibiting enhanced resistance to oxidation at lower cost would be a highly desirable material. Moreover, it would also be of considerable commercial advantage were these benefits to be obtained without adversely affecting other characteristics for which such prior art alloys are known, notably resistance to stress-corrosion cracking and good weldability. The present invention is therefore primarily directed to achieving these overall objectives.

It has now been discovered that specially proportioned, iron-nickel-chromium alloys containing correlated percentages of chromium, nickel, silicon and advantageously, cerium, exhibit extraordinary resistance to oxidation at elevated temperature and, in addition, are quite resistant to stress-corrosion cracking as well as being readily weldable.

It is an object of this invention to provide an iron-base alloy which is weldable and exhibits a high resistance to cyclic oxidation at elevated temperatures and good resistance to stress corrosion cracking.

It is another object of this invention to provide an electric heater element which is sheathed in an iron-base alloy characterized by excellent resistance to cyclic oxidation at elevated temperatures and good resistance to stress corrosion cracking.

Other objects and advantages will become apparent from the following description.

Generally speaking, the present invention contemplates weldable iron-base alloys composed of, by weight, from about 15% to about 23% nickel, from about 17% to about 23% chromium, from about 0.3% to about 1.5% silicon, cerium in a small but effective amount sufficient to improve oxidation and corrosion resistance, the cerium being up to about 0.05%, up to about 2% manganese, up to about 0.15% carbon, up to about 0.5% aluminum,

up to about 0.5% titanium, up to about 0.015% sulfur and the balance essentially iron. In addition it is important that the various constituents of the alloys be correlated so as to satisfy the following relationships which, upon being observed, result in high resistance to cyclic oxidation and good resistance to stress corrosion cracking, respectively:

1178—9986 (percent Ce)—1085 (percent Si)—49.78 (percent Cr)+3965 (percent Si $\times$ percent Ce)+304.5 (percent Cr $\times$ percent Ce)+44.84 (percent Si $\times$ percent Cr)+16.65 [percent Mn/(percent Si+percent Ce)] must be  $\leq 60$

—1156+109.1 (percent Ni)+2690 (percent Mn $\times$ percent Ce)—5.97 (percent Mn $\times$ percent Ni)—1.57 (percent Ni $\times$ percent Cr)+358.5 (percent Si $\times$ percent Cr) must be  $\geq 500$

Where the optimum of properties would not consistently be required, the cerium can be omitted, but even then it is much preferred to use, at least a small amount, e.g., 0.005%, for it has been found that in conjunction with silicon it counteracts the tendency for manganese to detract from oxidation resistance and resistance to stress corrosion cracking. Accordingly, these elements should be controlled such that the ratio percent Mn/(percent Si+percent Ce) has a value less than about 0.6 and the ratio percent Ni/percent Cr has a value in the range from 0.9 to 1.2. The alloys of the invention exhibit resistance to cyclic oxidation at 1800° F. equal to or superior to that of the sheathing alloys commonly used.

An advantageous composition of the alloy of the invention is composed of, by weight, about 20% nickel, about 20% chromium, about 0.6% silicon, about 0.02% cerium and the balance essentially iron except for small amounts of incidental elements and impurities including up to about 1% manganese.

In carrying the invention into practice, chromium and nickel promote resistance to oxidation, as well as resistance to general corrosion and to stress corrosion. Chromium in amounts in excess of about 23% has an adverse effect on workability. In general, the higher the chromium content within the specified range, the better the alloy produced, particularly with respect to oxidation resistance. Amounts of nickel beyond 23% are unnecessary and should the percentage fall much below 15% various characteristics can be adversely affected. In seeking the best combination of results a range of from 19% to 21% or 22% chromium and from about 18% to 22.5% nickel is quite satisfactory.

Silicon and cerium both aid in providing the required degree of oxidation and corrosion resistance. Silicon confers improved oxidation resistance; however, an amount of silicon above the range specified leads to problems in weldability, particularly hot cracking and excessive fluidity. A silicon content of from 0.6% or 0.7% to about 1% or 1.1% is deemed quite beneficial. Cerium is advantageously present in the alloys in the amount of from about 0.01% to about 0.05%.

The element cerium in amounts within the specified range makes an important contribution to the oxidation resistance and to stress corrosion resistance. It is good practice to include at least 0.01% cerium since the alloys are then less sensitive in respect of their corrosion resistance to variations in the amounts of the other alloy constituents, particularly, nickel, chromium, silicon and manganese. Quantities of cerium in excess of the specified range lead to difficulties in forging, rolling and in weldability. Thus, a cerium range of from 0.015% to about 0.04% is preferred.

The cerium which is employed in the alloys of this invention is ordinarily added as misch metal which also contains lanthanum and other rare earth elements. Typically, an addition of misch metal is composed, by weight,

of about 50% cerium, 20% lanthanum, with the balance other rare earth elements. It will be understood that in the alloys of this invention, where additions of cerium are made, there will usually also be several thousandths of a percent of lanthanum present.

The alloys of the invention may also include relatively small amounts of other elements which can be present as impurities without substantial detrimental effect. Such elements are contained in the alloys of the invention due to their unavoidable presence in the raw materials employed, or as a result of their use for one purpose or another during the preparation of the alloys. Thus, manganese in the amount of up to 2%, by weight, may be tolerated, but it is more advantageous to have no more than 1% present. Manganese in amounts in excess of the specified maximum has an adverse effect upon oxidation resistance and upon stress corrosion cracking. Up to about 0.15% by weight of carbon can be tolerated, but it is desirable that the alloy contain no more than about 0.1%. Excessive carbon may result in precipitation of carbides and hence, brittleness, which gives rise to problems in forming the alloy. It is quite difficult to obtain an alloy of this type which is entirely free from sulfur, and in this case up to 0.015% can be tolerated. Copper is also a common impurity which can be tolerated in amounts up to a maximum of 0.5%. Amounts of copper greater than this tend to reduce high temperature oxidation resistance. Aluminum, titanium and calcium are used as deoxidizers in melting the alloys of the invention, and residual amounts of these elements may remain in the final alloy composition. Thus, up to about 0.5% each, by weight, of aluminum and titanium may be present and in some cases, small amounts of calcium have been detected.

For the purpose of giving those skilled in the art a better appreciation of the advantages of the invention, the following illustrative examples are given.

### EXAMPLE

A number of heats of the alloys of the invention were prepared by charging appropriate amounts of iron, nickel and chromium into an air induction furnace and melting down the charge. Just before tapping the heat, the required silicon, aluminum, titanium and cerium additions (the latter in the form of misch metal) were added, and last of all, calcium. The heat was then poured into molds to produce 4 inch diameter ingots. The ingots thus prepared were forged into  $\frac{1}{4}$ -inch thick flat bars and then the flat bars were cold rolled to 0.125 inch thick sheet. Sections were cut from the sheet for use as cyclic oxidation specimens and for standard U-bend stress corrosion cracking test specimens and the remaining sections of the sheet were then welded end to end to make a roll of sheet which was then cold rolled to 0.025 inch thick sheet, the gauge commonly employed in making heater element sheathing. The following Table I gives the composition of a number of alloys which were prepared as described above.

TABLE II.—MECHANICAL PROPERTIES AT ROOM TEMPERATURE

[Material: Forged  $\frac{1}{4}$  inch square bar. Heat treatment: 1,800° F./1 hour; air cooled]

| Alloy No. | .2% Y.S.,<br>k.s.i. | T.S.,<br>k.s.i. | Elong.,<br>percent | R.A.,<br>percent | Hardness,<br>R <sub>B</sub> |
|-----------|---------------------|-----------------|--------------------|------------------|-----------------------------|
| 1-----    | 40.6                | 91.0            | 45.0               | 68.0             | 75                          |
| 2-----    | 38.5                | 82.7            | 48.0               | 68.5             | 74                          |
| 3-----    | 44.6                | 93.8            | 49.0               | 72.0             | 79                          |
| 4-----    | 37.0                | 87.3            | 49.0               | 72.6             | 73                          |
| 5-----    | 38.6                | 90.7            | 44.0               | 68.5             | 76                          |
| 6-----    | 34.8                | 90.8            | 45.0               | 68.0             | 76                          |
| 7-----    | 41.7                | 91.5            | 40.0               | 68.0             | 79                          |

The mechanical properties indicated in the above Table II for the alloys of the invention are quite comparable to the properties of the commonly employed prior art sheathing alloy referred to above herein. Such an alloy is produced to meet a sheet specification wherein the minimum tensile strength is 75,000 p.s.i., the minimum yield strength (0.2% offset) is 30,000 p.s.i., the minimum elongation is 30% and the maximum hardness is 80 R<sub>B</sub>.

In the following Table III, the depth of the oxidation attack on alloy sheet having a thickness of 0.125 inch and the weight loss sustained thereby is set forth under cyclic oxidation conditions wherein a test cycle was employed in which samples were heated to a temperature of 1800° F. in a furnace in air for 15 minutes, followed by 5 minutes cooling in air outside the furnace, such cycles being repeated for a period of 1,000 hours.

TABLE III.—OXIDATION ATTACK

| Alloy No. | Depth of<br>attack, in.* | Weight loss,<br>mg./cm. <sup>2</sup> |
|-----------|--------------------------|--------------------------------------|
| 1-----    | 0.001                    | 0                                    |
| 2-----    | 0.002                    | 9                                    |
| 3-----    | 0.001                    | 0                                    |
| 4-----    | 0.004                    | 19                                   |
| 5-----    | 0.003                    | 40                                   |
| 6-----    | 0.002                    | 0                                    |
| 7-----    | 0.003                    | 2                                    |

\*Original gauge—Remaining good metal

Depth of attack =  $\frac{2}{3}$

It will be observed from the above table that the alloys of the present invention, after 1,000 hours of test, have sustained relatively slight damage from oxidation attack. A commercial alloy of the composition described above and tested under the same conditions sustained oxidation damage to a depth of about 0.008 inch and a weight loss of over 120 mg./cm.<sup>2</sup>. Alloys which sustain a weight loss of up to 60 mg./cm.<sup>2</sup> in this oxidation test are considered to have exhibited high resistance to cyclic oxidation.

The alloys of Table I were also tested for resistance to stress corrosion cracking. Standard restrained U-bend stress corrosion cracking test specimens were prepared from alloy pieces which had the dimensions 6" x 0.5" x 0.125". The restrained test specimens were immersed in a boiling concentrated (45%) magnesium chloride solution and were periodically examined for cracking. When the tests were terminated after 720 hours (30 days) none

TABLE I.—CHEMICAL ANALYSIS OF ALLOYS

| Alloy No. | C    | Mn   | Fe   | S     | Si   | Cu   | Ni    | Cr    | Al    | Ti   | Ce    |
|-----------|------|------|------|-------|------|------|-------|-------|-------|------|-------|
| 1-----    | 0.05 | 0.41 | Bal. | 0.009 | 0.90 | 0.02 | 22.14 | 18.62 | 0.31  | 0.02 | 0.044 |
| 2-----    | 0.05 | 1.10 | Bal. | 0.005 | 0.71 | 0.02 | 20.27 | 20.37 | 0.11  | 0.12 | 0.022 |
| 3-----    | 0.04 | 0.08 | Bal. | 0.007 | 0.81 | 0.09 | 20.69 | 19.64 | 0.11  | 0.07 | 0.018 |
| 4-----    | 0.09 | 0.36 | Bal. | 0.008 | 0.93 | 0.02 | 18.02 | 17.63 | 0.38  | 0.22 | ----- |
| 5-----    | 0.11 | 1.63 | Bal. | 0.008 | 0.84 | 0.02 | 18.20 | 17.19 | 0.022 | 0.14 | 0.027 |
| 6-----    | 0.09 | 0.41 | Bal. | 0.008 | 1.03 | 0.02 | 22.06 | 22.72 | 0.004 | 0.19 | ----- |
| 7-----    | 0.09 | 1.80 | Bal. | 0.006 | 0.94 | 0.02 | 22.21 | 23.01 | 0.17  | 0.15 | 0.02  |

NOTE.—Bal.=balance iron plus impurities.

The tensile properties and hardness at room temperature of the alloys of Table I are set forth in the following Table II.

of the alloy specimens representing the alloys of Table I had failed whereas the commercial alloy mentioned above failed in just over 300 hours. It is considered that alloys

subjected to this test which survive 500 hours have exhibited good resistance to stress corrosion cracking. In this connection it is most advantageous that the ratio of nickel to chromium be at least unity, the silicon content should be 1% or more and the manganese should not exceed 0.5%.

The alloys of Table I were further tested for weldability by preparing autogenous TIG welds and examining the welds for cracking. The weldability of the alloys ranged from good to excellent.

A heat of commercial size has been produced having mechanical properties comparable to those set forth in Table II. This heat was made in a furnace having a nominal capacity of 5,000 pounds. The heat produced weighed roughly 5,500 pounds and had the following composition expressed in weight percent:

|                  |         |
|------------------|---------|
| Nickel -----     | 20.32   |
| Chromium -----   | 19.94   |
| Silicon -----    | 0.60    |
| Cerium -----     | 0.022   |
| Manganese -----  | 0.31    |
| Carbon -----     | 0.04    |
| Sulfur -----     | 0.007   |
| Phosphorus ----- | 0.010   |
| Aluminum -----   | 0.17    |
| Titanium -----   | 0.17    |
| Calcium -----    | 0.001   |
| Copper -----     | 0.03    |
| Iron -----       | Balance |

After forging, the heat was rolled to hot band  $\frac{1}{4}$ -inch thick, and thereafter cold rolled to the desired gauge of 0.090 inch. Cyclic oxidation and stress corrosion cracking test specimens were prepared and tested. The alloy exhibited a weight loss of only 3 mg./cm.<sup>2</sup> after 1000 hours of the cyclic oxidation test and standard U-bend specimens for the stress corrosion cracking test were exposed to test conditions for 720 hours without failure. Accordingly, this alloy clearly exhibits high resistance to cyclic oxidation and good resistance to stress corrosion cracking.

The alloys of the present invention also exhibit a resistance to general corrosion similar to that of Type 304 stainless steel. This property is of some importance in view of the fact that in normal use as sheathing alloys, they are often exposed to contact with various solutions at elevated temperature.

There has thus been disclosed a family of alloys having surprisingly good resistance to oxidation at elevated temperatures, though containing nickel in substantially smaller amounts than has been the practice in the art, particularly in the field of sheathing alloys for electrical heater elements. These alloys may also be usefully employed as heat exchangers and process piping, carburizing fixtures and retorts and furnace components.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A weldable, oxidation and corrosion-resistant alloy consisting essentially, by weight, of from about 15% to about 23% nickel, from about 17% to about 23% chromium, from about 0.3% to about 1.5% silicon, from a small but effective amount of cerium up to about 0.05% to improve oxidation and corrosion resistance, up to about 2% manganese, up to about 0.15% carbon, up to about 0.5% aluminum, up to about 0.5% titanium, up to about

0.015% sulfur and the balance essentially iron, which is characterized by exhibiting high resistance to cyclic oxidation resulting from balancing the constituents of the alloy within the ranges stated according to the following formula:

$$1178-9986 \text{ (percent Ce)} - 1085 \text{ (percent Si)} - 49.78 \\ (\text{percent Cr}) + 3965 \text{ (percent Si} \times \text{percent Ce)} + 304.5 \\ (\text{percent Cr} \times \text{percent Ce}) + 44.84 \text{ (percent Si} \times \text{percent Cr}) + 16.65 [\text{percent Mn}/(\text{percent Si} + \text{percent Ce})] \leq 60$$

10 and good resistance to stress corrosion cracking resulting from balancing the constituents of the alloy within the ranges stated according to the following formula:

$$-1156 + 109.1 \text{ (percent Ni)} + 2690 \text{ (percent Mn} \times \text{percent Ce)} - 5.97 \text{ (percent Mn} \times \text{percent Ni)} - 1.57 \\ (\text{percent Ni} \times \text{percent Cr}) + 358.5 \text{ (percent Si}^2) \geq 500$$

2. The alloy of claim 1 containing at least 0.01% cerium.

3. The alloy of claim 1 containing no more than 1% manganese.

4. The alloy of claim 1 containing from 18% to 22.5% nickel, from 19% to 22% chromium, from about 0.6% to about 1.1% silicon and from 0.015% to about 0.04% cerium.

25 5. The alloy of claim 2 wherein nickel is present in the amount of about 20, the chromium is present in the amount of about 20%.

6. The alloy of claim 3 wherein nickel is present in the amount of about 20%, and chromium is present in the amount of about 20%.

30 7. The alloy of claim 1 wherein the nickel is present in the amount of about 20%, chromium is present in the amount of about 20%, silicon is present in the amount of at least about 0.6% and cerium is present in the amount of about 0.02%.

8. The alloy of claim 1 wherein the ratio percent Ni/% Cr is at least unit, the silicon content is at least 1% and the manganese content does not exceed 0.5%.

40 9. A weldable, oxidation and corrosion-resistant alloy consisting essentially by weight, of from about 15% to about 23% nickel, from about 17% to about 23% chromium, from about 0.3% to about 1.5% silicon, from a small but effective amount of cerium up to about 0.05% to improve oxidation and corrosion resistance, up to about 45 2% manganese, up to about 0.15% carbon, up to about 0.5% aluminum, up to about 0.5% titanium, up to about 0.015% sulfur and the balance essentially iron, which is characterized by exhibiting high resistance to cyclic oxidation

50 resulting from balancing the constituents of the alloy within the ranges stated according to the following formula:

$$1178-9986 \text{ (percent Ce)} - 1085 \text{ (percent Si)} - 49.78 \\ (\text{percent Cr}) + 3965 \text{ (percent Si} \times \text{percent Ce)} + 304.5 \\ (\text{percent Cr} \times \text{percent Ce}) + 44.84 \text{ (percent Si} \times \text{percent Cr}) + 16.65 [\text{percent Mn}/(\text{percent Si} + \text{percent Ce})] \leq 60$$

55 10. The alloy of claim 9 containing at least 0.01% cerium.

#### References Cited

#### UNITED STATES PATENTS

|           |         |                 |          |
|-----------|---------|-----------------|----------|
| 2,174,919 | 10/1939 | Kay -----       | 75-128 E |
| 2,683,663 | 7/1954  | Tisdale -----   | 75-128 R |
| 2,738,267 | 3/1956  | Pakkala -----   | 75-124   |
| 2,687,954 | 8/1954  | Lohr -----      | 75-128 E |
| 3,362,813 | 1/1968  | Zolkowski ----- | 75-124   |

HYLAND BIZOT, Primary Examiner

70 U.S. Cl. X.R.

75-124, 128 T